

## UNITED STATES PATENT OFFICE.

HANS T. CLARKE AND CARL J. MALM, OF ROCHESTER, NEW YORK, ASSIGNEES TO  
EASTMAN KODAK COMPANY, OF ROCHESTER, NEW YORK, A CORPORATION OF NEW  
YORK.

## PROCESS OF REACETYLATING CELLULOSE ACETATE.

No Drawing.

Application filed January 12, 1927. Serial No. 160,766.

This invention relates to processes of reacetylation of cellulose acetate. One object of the invention is to provide a simple, inexpensive process for partly reacetylating cellulose acetate from which acetyl groups have been split off, such as by hydrolysis. Another object is to provide a simple and easily controlled process for adjusting or restoring the solubility of hydrolyzed cellulose acetate in organic solvents, such as acetone. Another object is to provide a process for restoring acetone-solubility in cellulose acetate which has been over-hydrolyzed to the point where such solubility has been impaired. Other objects will hereinafter appear.

Cellulose acetate has often been made by acetylating it as far as practical and thus obtaining chloroform-solubility. This product has then been hydrolyzed until a product is obtained which is soluble in acetone. Careful analysis has shown that the change from one solubility to the other is accomplished by a loss of acetyl groups during the hydrolysis. In other words, the acetone-soluble cellulose acetate contains less "combined acetic acid" than the chloroform-soluble species from which it was derived.

The hydrolysis may take place while the cellulose acetate is in solution in acetic acid, as in U. S. Reissue Patent No. 12,637, Miles, April 23rd, 1907, or it may take place by the hydrolysis of the solid cellulose acetate in an acid solution, as described, for example, in British Patent No. 24,067, Newton, of 1906. The solid cellulose acetate during this treatment may conveniently be in the form of a spray-dried powder, as explained in U. S. Patent No. 1,516,225, Webb, November 18th, 1924. A deacetylation action may also be brought about by a moderate saponification, as indicated in U. S. Patent No. 1,074,092, Mork, September 23rd, 1913, and No. 1,061,771, Mork, May 13th, 1913.

It is manifest that in all of these cases the action may be inadvertently carried too far. In the case of the acid treatment, either while the cellulose acetate is dissolved in acetic acid, or while it is in the form of solid par-

ticles, too long a treatment may greatly lessen, or even eliminate the solubility in acetone produced by the initial stages of the treatment. In the alkaline saponification the process may be carried so far that a reverted cellulose may be obtained. As the purpose of these processes was to obtain certain properties by splitting off part of the acetyl groups, it is undesirable to correct any excessive removal of the groups by replacing all of them. And yet a retreatment in the ordinary acetic acid-acetic anhydride-catalyst bath is practically sure to do this, giving, for example, a chloroform-soluble product. It is quite impractical, and very expensive, to carry such a reacetylation to only a partial degree,—for example, to restore normal acetone-solubility to cellulose acetate which has been rendered sparingly soluble in that liquid. Substantially a full acetylation must be obtained and then a second and correct hydrolysis carried out. It is manifestly desirable that there be some process which will, with accurate control, restore just enough of the removed acetyl groups to bring back the desired qualities or solubilities in the product, and to do this without the use of expensive ingredients, such as acetic anhydride.

We have found that the desired results may be obtained by heating the cellulose acetate, from which the acetyl groups have been split off, with acetic acid as the sole acetylating agent. This reintroduces acetyl groups in a positive manner and yet does it at a rate which places the proportion introduced under accurate control. For example, cellulose acetate, which has been hydrolyzed until the original acetyl percentage has dropped to the point where the product is no longer adequately soluble in acetone, can be restored to acetone-solubility by boiling in substantially anhydrous acetic acid for a moderate length of time of about the order of magnitude of 24 hours. Moreover, it may be rendered also soluble in chloroform by restoring substantially most of the acetyl groups upon boiling in acetic acid for a time of the order of magnitude of 200 hours,

This same treatment will acetylate cellulose acetates from which the acetyl groups have been even entirely removed.

It is well known that different batches of cellulose acetate vary somewhat in their susceptibilities toward different solvents, but the specimen referred to in the following table illustrates a common type.

| 10 | Per cent acetyl | Chloroform      | Acetone          | Warm ethyl alcohol |
|----|-----------------|-----------------|------------------|--------------------|
| 15 | 44.8            | Soluble.        | Insoluble.       | Insoluble.         |
|    | 42.0            | Soluble.        | Partly soluble.  | Insoluble.         |
|    | 40.1            | Soluble.        | Soluble.         | Insoluble.         |
|    | 38.9            | Partly soluble. | Soluble.         | Insoluble.         |
|    | 37.1            | Partly soluble. | Readily soluble. | Partly soluble.    |
|    | 35.2            | Insoluble.      | Readily soluble. | Partly soluble.    |
|    | 34.2            | Insoluble.      | Partly soluble.  | Partly soluble.    |
|    | 32.8            | Insoluble.      | Insoluble.       | Soluble.           |
|    | 31.1            | Insoluble.      | Insoluble.       | Soluble.           |

20 The first column shows the percentage of acetyl group which is present in the cellulose acetate, as the hydrolysis with acids progresses. The second column shows how the solubility in chloroform diminishes and disappears as the percentage of acetyl groups drops. The third column shows how the solubility in acetone grows to a maximum and then diminishes until it disappears. The fourth column shows the development of solubility in warm ethyl alcohol. This illustrates changes which may be brought about by ordinary methods of hydrolysis. It is apparent that carelessness or inadvertence may cause the hydrolysis 35 to be prolonged to a point where the desired solubility, say in acetone, is impaired or even lost altogether.

Our process may then be used for restoring desired solubility by restoring or replacing 40 at least some of the acetyl groups. For example, a cellulose acetate, which was originally soluble in chloroform, but not in acetone, and contained nearly 45% of acetyl groups, was hydrolyzed by acids in the well known way until it contained only 31.2% of acetyl groups and had become entirely insoluble in either acetone or chloroform. One part of this was boiled, at atmospheric 50 pressure, with 20 parts by weight of acetic acid. After 24 hours boiling the product contained 37.3% of acetyl groups and was readily soluble in acetone and partially soluble in chloroform. This brought it to the stage where it was in its best commercial 55 form as regards acetone-solubility. A similar process conducted for 48 hours, on the same sample, brought about an acetyl content of 40.5% thus giving a fair solubility in both chloroform and acetone. The process 60 was carried out on the same sample for 200 hours until it contained 42.3% of acetyl groups with the same solubilities. It will be apparent that this process proceeds at such a rate that samples can readily be withdrawn and tested and the action stopped

at the desired stage, thus very accurately gauging the amount of acetyl groups restored to each molecule of cellulose acetate. It will be noted that the acetic acid is the sole acetylating agent and we do not require 70 the use of expensive acetic anhydrid, or even the use of a catalyst.

When working at atmospheric pressure the acid is boiled and thus the reaction carried on at about 117° C. It proceeds at a 75 useful rate, however, even at somewhat lower temperatures, preferably above 100° C. Moreover, higher temperatures may be employed when superatmospheric pressure is employed. As a general proposition, we 80 prefer to keep the temperatures below 170° C. in order to avoid molecular degradation of the products, as evidenced by the brittleness of films formed from them. When superatmospheric pressure is employed, the 85 time to produce a given reacetylation is reduced. But the process proceeds at a satisfactory rate when the acid is boiled at atmospheric pressure, and this is the preferred form.

It is desirable to use substantially anhydrous acid and to remove at least some of the water formed during the reaction. These conditions are satisfactorily met by using a fractional reflux condenser, which 95 will condense and return to the bath the vapors of acetic acid without condensing the water vapor.

Having thus described our invention, what we claim as new and desire to secure by Letters Patent is:

1. The process of at least partially reacetylating cellulose acetate from which at least part of the acetyl groups have been removed until its solubility has thereby been 105 impaired, which comprises heating said cellulose acetate with acetic acid as the sole acetylating agent until further acetyl groups are introduced to correct said impaired solubility, the temperature being kept below the 110 decomposition point of the product.

2. The process of at least partially reacetylating cellulose acetate, the solubility of which has been changed by removal of acetyl groups by hydrolysis, which comprises heating said cellulose acetate with acetic acid as the sole acylating agent to temperatures above 100° C. but below 170° C. until acetyl groups are introduced to replace those removed and restore the solubility which existed before said removal.

3. The process of correcting the solubility of cellulose acetate, formed by excessive hydrolysis of chloroform-soluble cellulose acetate until acetone-solubility is produced and then impaired, which comprises heating said hydrolyzed acetate with acetic acid as the sole acetylating agent between 100° C. and 170° C. until acetyl groups are introduced to correct said impaired acetone-solubility.

4. The process of partially reacetylating cellulose acetate, the solubility of which has been changed by removal of acetyl groups by hydrolysis, which comprises boiling said cellulose acetate at atmospheric pressure with substantially anhydrous acetic acid with fractional refluxing condensation, to

remove water formed by the reaction, until acetyl groups are introduced to replace those removed and restore the solubility. <sup>10</sup>

Signed at Rochester, New York, this 7th day of January, 1927.

HANS T. CLARKE.  
CARL J. MALM.